



US006342289B1

(12) **United States Patent**  
Eguchi et al.

(10) **Patent No.:** US 6,342,289 B1  
(45) **Date of Patent:** \*Jan. 29, 2002

(54) **RECORDING MEDIUM, PROCESS FOR PRODUCTION THEREOF, AND INK-JET RECORDING METHOD EMPLOYING THE MEDIUM**

(75) Inventors: **Takeo Eguchi**, Tokyo; **Kyo Miura**, Yokohama; **Hitoshi Yoshino**, Zama, all of (JP)

(73) Assignee: **Canon Kabushiki Kaisha**, Tokyo (JP)

(\*) Notice: This patent issued on a continued prosecution application filed under 37 CFR 1.53(d), and is subject to the twenty year patent term provisions of 35 U.S.C. 154(a)(2).

Subject to any disclaimer, the term of this patent is extended or adjusted under 35 U.S.C. 154(b) by 0 days.

(21) Appl. No.: **08/771,910**

(22) Filed: **Dec. 23, 1996**

**Related U.S. Application Data**

(62) Division of application No. 08/528,208, filed on Sep. 12, 1995, now abandoned.

(30) **Foreign Application Priority Data**

Sep. 16, 1994 (JP) ..... 6-221496  
Aug. 31, 1995 (JP) ..... 7-223694

(51) **Int. Cl.<sup>7</sup>** ..... **B41M 5/00**

(52) **U.S. Cl.** ..... **428/195; 428/328; 428/329**

(58) **Field of Search** ..... **428/195, 328, 428/329**

(56) **References Cited**

**U.S. PATENT DOCUMENTS**

|             |         |                 |       |           |
|-------------|---------|-----------------|-------|-----------|
| 4,202,870 A | 5/1980  | Weber et al.    | ..... | 423/630   |
| 4,242,271 A | 12/1980 | Weber et al.    | ..... | 260/448   |
| 4,474,847 A | 10/1984 | Schroder et al. | ..... | 428/323   |
| 4,879,166 A | 11/1989 | Misuda et al.   | ..... | 428/212   |
| 4,946,666 A | 8/1990  | Brown           | ..... | 423/625   |
| 5,104,730 A | 4/1992  | Misuda et al.   | ..... | 428/304.4 |

5,122,814 A 6/1992 Endo et al. ..... 346/33 R  
5,306,680 A \* 4/1994 Fukuda ..... 501/153  
5,463,178 A \* 10/1995 Suzuki et al. ..... 428/195

**FOREIGN PATENT DOCUMENTS**

|    |              |           |
|----|--------------|-----------|
| DE | 3024205 A1   | 1/1982    |
| EP | 0500021 A1   | 8/1992    |
| EP | 0 634 287 A1 | 1/1995    |
| JP | 54-59936     | 5/1979    |
| JP | 56-76246     | 6/1981    |
| JP | 56-95985     | 8/1981    |
| JP | 2-276670     | 11/1990   |
| JP | 01-64499     | * 12/1990 |
| JP | 4-37576      | 2/1992    |
| JP | 5-32037      | 2/1993    |

**OTHER PUBLICATIONS**

The Journal of the American Chemical Society vol. LXXIII, date Jan.-Mar. 1951, pp. 373-380.

The Journal of the American Chemical Society vol. LX, dated Jan.-Jun. 1938, pp. 309-319.

\* cited by examiner

*Primary Examiner*—Pamela R. Schwartz

(74) *Attorney, Agent, or Firm*—Fitzpatrick, Cella, Harper & Scinto

(57)

**ABSTRACT**

In a recording medium having a porous ink-receiving layer containing alumina hydrate of boehmite structure formed on a base material, the alumina hydrate has crystallinity ranging from 15 to 80 and microcrystals of the alumina hydrate are directed to be parallel to a plane direction of the ink-receiving layer at a parallelization degree of not less than 1.5. The recording medium is employed in an ink-jet recording method conducting printing by ejecting ink droplets through an orifice onto the recording medium.

A process for producing the recording medium comprises the steps of: applying a coating liquid containing alumina hydrate of boehmite structure with shearing stress onto a base material; and drying the coated material to obtain a degree of parallelization of a microcrystal of the alumina hydrate with a plane direction of the ink-receiving layer of not less than 1.5.

**7 Claims, 2 Drawing Sheets**



← →  
**PLANE DIRECTION OF THE INK-RECEIVING LAYER**

FIG. 1



FIG. 2A



← →  
PLANE DIRECTION  
OF  
THE INK-RECEIVING LAYER

FIG. 2B



FIG. 2C



FIG. 2D



FIG. 3A



FIG. 3B



**RECORDING MEDIUM, PROCESS FOR  
PRODUCTION THEREOF, AND INK-JET  
RECORDING METHOD EMPLOYING THE  
MEDIUM**

This application is a division of Application Ser. No. 08/528,208 filed Sep. 12, 1995, now abandoned.

**BACKGROUND OF THE INVENTION**

1. Field of the Invention

The present invention relates to a recording medium suitable for recording with aqueous ink, particularly to a recording medium suitable for ink-jet recording.

2. Related Background Art

Ink jet recording is a method for recording images and letters by ejecting fine droplets of ink onto a recording medium such as a paper a sheet. Ink jet recording is rapidly becoming popular in recent years for various applications because of its high recording speed, ease of multicolor recording, flexibility in pattern recording, and because image fixation is not needed. Multicolor ink-jet recording is coming to be used in full color image recording since it is capable of giving images comparable with images formed by multicolor gravure printing or color photography, and is less expensive than multicolor printing when the number of reproduction is small. With improvements in recording speed, fineness of recording, and full color recording, the recording medium is required to have better qualities in addition to the improvements of the recording apparatus and the recording method.

Hitherto, various types of recording mediums have been disclosed. For example, recording sheets having a layer containing alumina hydrate of pseudo boehmite structure are disclosed in U.S. Pat. Nos. 4,879,166 and 5,104,730, and Japanese Patent Laid-Open Application Nos. 2-276670, 4-37576, and 5-32037. The prior art recording mediums involve disadvantages as follows: occurrence of beading of ink dots, due to insufficient absorbency for a large amount of ink in color image printing; likelihood of being scratched by a sheet delivery device due to insufficient surface hardness; likelihood of the ink-receiving layer surface cracking due to insufficient bonding strength of the ink-receiving layer; low circularity of printed dots cracking due to insufficient uniformity of the ink-receiving layer; and low gloss of recording medium due to less orientation of the pigment.

The beading mentioned in the present invention refers to a phenomenon in which dots irregularly move in the plane direction of the surface of an ink-receiving layer when the ink is still fluid before it is fixed in the ink-receiving layer.

The present invention has been made to offset the above disadvantages.

**SUMMARY OF THE INVENTION**

An object of the present invention is to provide a recording medium which has high ink absorbency to absorb ink at a higher absorbing rate and having higher surface hardness to be less liable to cracking on the surface.

Another object of the present invention is to provide a recording medium which is capable of forming an image with high circularity of dots and high gloss of the recorded image.

A still another object of the present invention is to provide a recording medium which provides water fastness and light fastness of the recorded image with less migration of the ink, in addition to the aforementioned properties.

A further object of the present invention is to provide a process for producing the aforementioned recording medium.

5 A still further object of the present invention is to provide an ink-jet recording method employing the aforementioned recording medium.

According to an aspect of the present invention, there is provided a recording medium having a porous ink-receiving layer containing alumina hydrate of boehmite structure formed on a base material, the alumina hydrate having 10 crystallinity ranging from 15 to 80.

According to another aspect of the present invention, there is provided a recording medium having a porous ink-receiving layer containing alumina hydrate of boehmite structure formed on a base material, wherein microcrystals of the alumina hydrate are directed to be parallel to the plane direction of the ink-receiving layer at a parallelization degree of not less than 1.5.

According to still another aspect of the present invention, there is provided a recording medium having a porous ink-receiving layer containing alumina hydrate of boehmite structure formed on a base material, the alumina hydrate having crystallinity ranging from 15 to 80, and the microcrystals of the alumina hydrate being directed to be parallel to the plane direction of the ink-receiving layer at a parallelization degree of not less than 1.5.

According to a further aspect of the present invention, there is provided an ink-jet recording method employing the above recording medium.

According to a still further aspect of the present invention, 30 there is provided a process for producing a recording medium having a porous ink-receiving layer containing alumina hydrate of boehmite structure, comprising the steps of: applying a coating liquid containing alumina hydrate of boehmite structure with shearing stress onto a base material; and drying the coated material to obtain the degree of 35 parallelization of the microcrystal of the alumina hydrate with the plane direction of the ink-receiving layer of not less than 1.5.

According to a still further aspect of the present invention, 40 there is provided a process for producing a recording medium, comprising the steps of: applying a liquid dispersion containing alumina hydrate of boehmite structure having crystallinity ranging from 15 to 80 onto a base material; and drying the coated material at a relative humidity of 20 45 to 60% to obtain crystallinity of the alumina hydrate ranging from 15 to 80 in the recording medium.

According to a still further aspect of the present invention, 50 there is provided a process for producing a recording medium, comprising the steps of: applying a liquid dispersion containing alumina hydrate of boehmite structure having crystallinity of lower than 15 onto a base material; and drying the coated material at a relative humidity of 10 to 20% to obtain crystallinity of the alumina hydrate ranging from 15 to 80 in the recording medium.

55 According to a still further aspect of the present invention, there is provided a process for producing a recording medium comprising the steps of: applying a liquid dispersion containing alumina hydrate of boehmite structure having crystallinity of lower than 15 on a base material; and heating the coated material at a relative humidity of 10 to 20% to obtain crystallinity of the alumina hydrate ranging from 15 to 80 in the recording medium.

**BRIEF DESCRIPTION OF THE PREFERRED  
EMBODIMENTS**

65 FIG. 1 is a schematic sectional view for explaining a recording medium of the present invention.

FIGS. 2A to 2D are schematic sectional views for explaining the degree of parallelization of the microcrystals in the recording medium of the present invention.

FIGS. 3A and 3B are schematic sectional views for explaining the dependency of ink absorbing rate on the direction of the planes (020) of microcrystalline alumina hydrate in the recording medium of the present invention.

#### DESCRIPTION OF PREFERRED EMBODIMENTS

The recording medium according to the present invention exhibits high ink absorbency, absorbs ink at a high rate, has sufficient surface hardness, is less liable to cause cracking of the surface, provides high circularity of printed dots, and has high gloss. The recording medium provides good water fastness and good light-fastness to the recorded matter with less migration of the recording liquid.

The recording medium of the present invention, in an embodiment, has one ink-receiving layer 2 of a porous structure comprising alumina hydrate and a binder provided on a base material 1.

The alumina hydrate, which is positively charged, is preferred as the constituting material for the ink-receiving layer, since it fixes the applied ink by a positive charge to give excellent colors to images, and does not involve the disadvantages of browning of black ink and low light-fastness which are problems associated with the use of a silica type compound for the ink-receiving layer. Of the alumina hydrates, one having boehmite structure is more suitable because of high adsorbability of dyes, high absorbency of ink, and high transparency.

The alumina hydrate contained in the recording medium of the present invention is defined by the general formula below:



where n is an integer of zero to 3, and m is a number of from zero to 10, preferably from zero to 5. In many cases, "mH<sub>2</sub>O" expresses a free water phase which does not contribute to the construction of a crystal lattice and is releasable. Therefore, the value of "m" is not necessarily an integer. The value of "m" may become zero when the alumina is calcined.

The process for producing the alumina hydrate having a boehmite structure to be incorporated into the recording medium of the present invention is not specially limited. The process includes Bayer process, alum pyrolysis process, and other processes for producing alumina hydrate. A suitable process is hydrolysis of a long-chain alkoxide of aluminum by addition of an acid. The long-chain alkoxide herein means alkoxides of 5 or more carbons, more preferably alkoxides of 12 to 22 carbons. With such an aluminum alkoxide, removal of the alcohol component and control of the shape of the alumina hydrate of boehmite structure are facilitated. The above-mentioned processes are advantageous because of less likelihood of contamination by ions and other impurities in comparison with processes using alumina hydrogel or cationic alumina. Further, long-chain alkoxides of aluminum are advantageous in that the alcohol resulting from the hydrolysis can readily be removed completely from the alumina hydrate in comparison with short-chain alkoxides such as aluminum isopropoxide.

The alumina hydrate prepared by the above process may be subjected to hydrothermal synthesis to allow the particles to grow, or may be dried to obtain powdery alumina hydrate.

In the present invention, a liquid dispersion containing the alumina hydrate and a binder is applied onto a base material,

and the applied matter is subjected to drying and other treatments to form a recording medium having a porous ink-receiving layer. The properties of the recording medium depend on the alumina hydrate employed, the liquid dispersion, and the conditions of production such as coating application and drying. In the present invention, it was found that the ink absorbency of the porous ink-receiving layer can be improved and the cracking thereof can be prevented by control of the crystallinity and the parallelization degree of the alumina hydrate in the layer.

The crystallinity in the present invention is defined as follows:

As shown in FIG. 2A, particles of alumina hydrate 6 having boehmite structure contained in the ink-receiving layer 2 are constituted of non-crystalline portions 10 and crystalline portions (boehmite microcrystals) 3.

The crystallinity degree means the ratio of crystalline portion to the entire alumina hydrate having a boehmite structure. The crystallinity is derived from an X-ray diffraction pattern measured by CuK $\alpha$  line of the pulverized ink-receiving layer, from the ratio of the peak intensity of the plane (020) appearing at about 20=14°-15° to the peak intensity at 20=10°. The crystallinity is disclosed in Japanese Patent Laid-Open Application Nos. 56-76246 and 56-95985.

In the present invention, the crystallinity of the alumina hydrate in the ink-receiving layer is preferably in the range of from 15 to 80. Within this range, the ink absorbency and the ink absorbing rate are satisfactory. More preferably, the crystallinity ranges from 20 to 70. Within this range, the surface hardness is higher, and the cracking is less likely to occur. At a crystallinity lower than 15, the ink absorbency and the ink absorbing rate are insufficient, whereas at a crystallinity higher than 80, the affinity to water is lower, which makes beading of ink dots likely to occur.

The parallelization degree in the present invention is defined as follows. As shown in FIG. 2A, the parallelization degree relates to the ratio of fine boehmite crystals 3 having (020) planes parallel to the plane direction of the ink-receiving layer to the entire fine boehmite crystals contained in the ink-receiving layer. FIG. 2D shows the plane direction of alumina hydrate fine crystals drawn in FIGS. 2A, 2B and 2C. The alumina hydrate has planes (020) 4 and planes (120) 5 as shown in FIG. 2D.

To measure the parallelization degree, the ratio of the intensities of X-ray diffraction peaks measured by CuK $\alpha$  line of plane (020) to that of plane (120) is derived for the ink-receiving layer (Ratio A); and separately the same ratio is derived for the pulverized ink-receiving layer (Ratio B). The parallelization degree is represented by the ratio of Ratio A to Ratio B.

When the planes (020) are directed completely at random, the parallelization degree of the ink-receiving layer is 1. As shown in FIGS. 2A to 2C, a higher parallelization degree means a higher ratio of the plane (020) parallel to the ink-receiving layer face. The parallelization degrees in FIGS. 2A, 2B and 2C are low, moderate, and high, respectively.

The recording medium of the present invention has a parallelization degree of preferably not less than 1.5 to obtain a higher circularity of the printed dots. If the parallelization degree is less than 1.5, the circularity of the printed dots is low. The parallelization degree is more preferably 2 or higher, thereby making the gloss of the recording medium higher.

The mechanism of ink absorption in the recording medium of the present invention is assumed to be described

as below. The ink droplets deposited on the surface of the recording medium are absorbed mainly by the interspaces between the planes (020) in the alumina hydrate particles. In a recording medium having a low parallelization degree as shown in FIG. 3A, the deposited ink diffuses non-uniformly due to random orientation of the crystal planes (020) in the ink-receiving layer face direction. On the other hand, in a recording medium having a high parallelization degree as shown in FIG. 3B, the ink diffuses uniformly in the recording layer face direction. Thereby, the circularity of the printed dots is presumed to be higher in the recording medium having the parallelization degree of 1.5 or more. In FIGS. 3A and 3B, the numeral 7 indicates a microcrystal of alumina hydrate particle into which ink 8 has penetrated. The numeral 9 indicates a printing head of the printer.

The light refractivity of the alumina hydrate at the crystalline portion differs from that at the non-crystalline portion. Therefore, the recording medium having randomly oriented crystal plane (020) of the alumina hydrate exhibits more noticeable light scattering than one having uniformly oriented planes (020). Therefore, a recording medium having a parallelization degree of 2 or higher exhibits lower light scattering and has higher gloss, presumably.

The recording medium, which has crystallinity of the alumina hydrate of from 15 to 80 and a parallelization degree of the alumina hydrate microcrystal of 1.5 or higher, has high water resistance and high light-fastness, and does not cause migration of the dye during storage, desirably. When the crystallinity is outside the above range, the affinity of the recording medium to the ink is lower, which causes migration repulsion, and beading of the ink, and retards the ink absorption. With the parallelization degree outside the above range, migration of the ink is likely to occur, due to the lower bonding strength of the dye to the recording medium. The dye of the ink is adsorbed by the interspaces between the crystal planes (020) of alumina hydrate microcrystals. The adsorbed dye is less releasable in the recording medium having higher parallelization degree due to higher adsorption strength caused by interaction of the uniformly orientated alumina crystal planes (020). This is because the recording medium having a higher parallelization degree has a lot of alumina microcrystal planes (020), whereby many adsorbing points are provided therein, and if the recording medium has a higher parallelization degree too, the planes (020) are uniformly oriented. Therefore, the above-mentioned effects can be obtained with the recording medium having the crystallinity and parallelization degree in the aforementioned ranges.

The aforementioned Japanese Patent Laid-Open Application No. 2-276670 describes a recording medium employing an agglomerate of fine alumina particle oriented in one direction which is formed by orienting particles of alumina hydrate, and has a constitution different from the recording medium having a specified parallelization degree of the planes (020) of the present invention. Furthermore, this Japanese Patent Laid-Open Application does not mention the circularity and the gloss which are the effects of the present invention, and is based on the idea different from the present invention.

The crystallinity of the alumina hydrate in the recording medium can be changed by controlling the heating conditions in drying the alumina hydrate-containing dispersion, and the parallelization degree can independently be changed by shearing stress on application of the dispersion.

The crystallinity of the alumina hydrate employed in the present invention is preferably in the range of from 15 to 80, since crystallinity within this range can be attained easily.

The alumina hydrate which has a crystallinity of less than 15 can be changed to have higher crystallinity in later processing. The alumina hydrate may be in a needle shape or in a plate shape. The particle size of the alumina hydrate is preferably in the range of from 1 to 50 nm in the maximum length for a needle-shaped particle or in the maximum diameter for a plate-shaped particle, since the viscosity of the dispersion is low and cracking or powder-falling is less likely to occur in this particle size range. The alumina hydrate has preferably a pore volume ranging from 0.1 to 1.0 cm<sup>3</sup>/g, and a pore radius ranging from 2.0 to 20.0 nm in view of ink absorbency. The specific surface area of the alumina hydrate ranges preferably from 10 to 500 m<sup>2</sup>/g in view of the low haze of the ink receiving layer for obtaining a glossy image and for observing an image by transmitted light.

The recording medium of the present invention can be prepared by applying a liquid dispersion containing the alumina hydrate and a binder onto a base material. By controlling the shearing stress in a specified range on application of the liquid dispersion onto the base material, the microcrystal planes (020) can be oriented in the direction parallel to the flow of the coating liquid dispersion, whereby the recording medium is made to have a high parallelization degree. The required shearing stress depends on the coating method and the viscosity of the liquid dispersion, and ranges preferably from 0.1 to 20.0 N/m<sup>2</sup>. In this range of shearing stress, microcrystals of the alumina hydrate are oriented to have a parallelization degree of 1.5 or more. When the shearing stress is lower than the above range, it is difficult to make the parallelization degree 1.5 or higher. With the shearing stress higher than the above range, the resulting ink-receiving layer tends to be non-uniform in thickness.

The coating may be conducted by any method, provided that the shearing stress in the above range can be applied. The preferred coating method includes kiss-roll coating, extrusion coating, slide hopper coating, curtain coating, blade coating, brush coating, bar coating, and gravure coating.

The suitable coating speed depends on the coating method. With a coating method in which the shearing stress depends on the coating speed, such as kiss-roll coating, extrusion coating, slide hopper coating, curtain coating, and bar coating, the coating speed ranges preferably from 0.01 to 10 m/s. At a coating speed of lower than 0.01 m/s, little shearing stress will be applied, and the parallelization degree tends to be lower. At a coating speed of higher than 10 m/s, the thickness of the ink-receiving layer is not readily controllable uniformly. The viscosity of the liquid dispersion at the time of the coating ranges preferably from 10 to 500 mPa·s. At a viscosity of lower than 10 mPa·s, the shearing stress given to the liquid dispersion is lower, and thereby the parallelization degree of alumina hydrate microcrystals in the resulting recording medium tends to be lower. At a viscosity of higher than 500 mPa·s, the thickness of the ink-receiving layer is not readily controllable uniformly. The amount of the coating of the liquid dispersion ranges preferably from 2 to 60 g/m<sup>2</sup> in terms of the dried solid matter.

The liquid dispersion after coating application is dried, preferably without blowing of drying air thereon, at least for one second to be thickened and set in an oriented state of the microcrystal planes (020) of the alumina hydrate by utilizing thixotropy of the liquid dispersion. If drying air is blown on the unset coating layer, it displaces the particles of the alumina hydrate and destroys the oriented state of the crystal planes (020) of the alumina hydrate which were made by the shearing stress, resulting in a low parallelization degree.

The applied coating liquid dispersion containing the alumina hydrate forms the ink-receiving layer by heat-drying.

It was found that the crystallinity can be controlled to be within the above specified range by controlling the heating rate, drying temperature, and drying time. Particularly, the crystallinity depends on the drying speed.

Therefore, the crystallinity can be controlled within the above range by controlling the humidity, temperature and drying time in the process of drying the liquid dispersion. When the recording medium is prepared from alumina hydrate having a crystallization degree of from 15 to 80 dispersed in a coating liquid dispersion, drying at a relative humidity ranging from 20% to 60% gives the alumina hydrate in the resulting recording medium a crystallinity in the above specified range. Drying at a relative humidity lower than 20% makes it difficult to control the crystallinity of the recording medium because of the large change in the crystallinity of the alumina hydrate per unit time. Drying at a relative humidity higher than 60% tends to cause non-uniform thickness of the ink-receiving layer because of the lower drying speed of the coating film.

When the recording medium is prepared from alumina hydrate having a crystallization degree of lower than 15 dispersed in a coating liquid dispersion, drying at a relative humidity ranging from 10% to 20% gives the crystallinity of the alumina hydrate in the resulting recording medium in the above specified range. Further, an alternative process can be provided, which comprises applying onto a base material a liquid dispersion containing alumina hydrate having crystallinity of lower than 15, followed by drying the liquid dispersion to form an ink receiving layer, and heating the obtained recording medium at a relative humidity of 10 to 20%, whereby it is possible to control the crystallinity within the above-mentioned range. Drying at a relative humidity lower than 10% makes it difficult to control the crystallinity to be not higher than 80 because of the rapid rise in the crystallinity of the alumina hydrate per unit time. In this case, it is also likely to generate cracking. Drying at a relative humidity of higher than 20% does not result in the intended crystallinity because of lack of increase in the crystallinity.

The most suitable heat-drying conditions (temperature and time) depend on the composition of the coating liquid, but are generally a heating temperature ranging from 60° C. to 150° C., and a heating time ranging from 2 seconds to 30 minutes. It is difficult to achieve the crystallinity in the above specified range at a drying temperature of lower than 60° C. even at the aforementioned humidity range. At a drying temperature higher than 150° C., the crystallinity will exceed the above specified range due to excessively high drying speed, and furthermore the ink-receiving layer is likely to be cracked. At a drying time of less than 2 seconds, the formed ink-receiving layer will become non-uniform in layer thickness because of insufficient drying time. A drying time of longer than 30 minutes is not effective since the change of the crystallinity will be finished within 30 minutes.

The above heating process can be conducted with a drying apparatus including hot air driers such as a direct tunnel drier, an arch drier, an air loop drier, and a sine-curve air float drier; infrared heating driers; microwave driers; and heating rolls.

The binder which may be used with the alumina hydrate in the present invention may be selected from water-soluble polymers, including preferably polyvinyl alcohol and modifications thereof (cation-modified, anion-modified, and silanol-modified), starch and modifications thereof (oxidized, and etherified), gelatin and modifications thereof, casein and modifications thereof, gum arabic, cellulose

derivatives such as carboxymethylcellulose, hydroxyethylcellulose, and hydroxypropylmethylcellulose, SBR latexes, NBR latexes, diene type copolymer latex such as methyl methacrylate-butadiene copolymer latex, functional group-modified polymer latexes, vinyl copolymer latexes such as ethylene-vinyl acetate copolymer latex, polyvinylpyrrolidones, maleic anhydride copolymers, acrylic ester copolymers, and the like.

The mixing weight ratio of the alumina hydrate having boehmite structure to the binder ranges preferably from 5:1 to 25:1. Within this range, the cracking or the powder-falling of the ink-receiving layer can be prevented. The mixing weight ratio ranges more preferably from 5:1 to 20:1. Within this range, cracking can be prevented which is caused by folding of the recording medium.

To the pigment and the binder, there may be added a pigment dispersant, a viscosity increaser, a pH controller, a lubricator, a fluidity modifier, a surfactant, an antifoaming agent, water-proofing agent, a foam inhibitor, a releasing agent, a foaming agent, a penetrating agent, a coloring dye, a fluorescent whitener, an ultraviolet absorber, an antioxidant, an antiseptic agent, a mildewproofing agent, and the like. The water-proofing agent may be selected from known materials such as quaternary ammonium salts, and polymeric quaternary ammonium salts.

The base material may be a paper sheet such as a sized paper sheet, a non-sized paper sheet, or a resin-coated paper; a sheet-shaped material such as a thermoplastic resin film; or cloth. The thermoplastic resin film may be a transparent film of a resin such as polyester, polystyrene, polyvinyl chloride, polymethyl methacrylate, cellulose acetate, polyethylene, or polycarbonate; or a pigment-filled or finely-foamed opaque plastic sheet.

The ink-receiving layer constituting the recording medium of the present invention has a total pore volume ranging preferably from 0.1 to 1.0 cm<sup>3</sup>/g. With the pore volume larger than a above range, the ink-receiving layer is likely to cause cracking or powder-falling therefrom. With the pore volume smaller than the above range, the ink-receiving layer exhibits low ink-absorbency, and is likely to cause migration of ink on the ink-receiving layer particularly in multicolor printing.

The ink-receiving layer has a BET specific surface area preferably ranging from 20 to 450 m<sup>2</sup>/g. With a specific surface area smaller than this range, the ink-receiving layer is not glossy, and has a high haze which gives a hazed image. With a specific surface area larger than the above range, the ink-receiving layer is likely to crack. The aforementioned BET specific surface area and the pore volume are measured, after degassing treatment at 120° C. for 24 hours, by a nitrogen adsorption-desorption method.

The ink employed in the recording according to the present invention comprises a coloring material (dye or pigment), a water-soluble organic solvent, and water as the main constituents. The dye is preferably a water-soluble dye such as a direct dye, acid dye, basic dye, reactive dye, or food dye. Any dye may be used, provided that it has the required properties such as fixability, color-developability, sharp image formation, stability, and light-fastness in combination with the recording medium.

The water-soluble dye is generally used as a solution in water or a mixed solvent of water and an organic solvent. The solvent is preferably a mixture of water and a water-soluble organic solvent. The water content in the ink ranges preferably from 20% to 90%, more preferably from 60% to 90% by weight.

The aforementioned water soluble organic solvent includes alkyl alcohols of 1 to 4 carbons such as methyl

alcohol, ethyl alcohol, n-propyl alcohol, isopropyl alcohol, n-butyl alcohol, s-butyl alcohol, t-butyl alcohol, and isobutyl alcohol; amides such as dimethylformamide, and dimethylacetamide; ketones and ketone alcohols such as acetone, and diacetone alcohol; ethers such as tetrahydrofuran, and dioxane; polyalkylene glycols such as polyethylene glycol, and polypropylene glycol; alkylene glycols having an alkylene group of 2 to 6 carbons such as ethylene glycol, propylene glycol, 1,2,6-hexanetriol, thioglycol, hexylene glycol, and diethylene glycol; glycerol; lower alkyl ethers of polyhydric alcohols such as ethylene glycol methyl ether, diethylene glycol monomethyl ether, diethylene glycol ethyl ether, triethylene glycol monomethyl ether, and triethylene glycol monoethyl ether; and the like.

10  
15  
20  
25  
30  
35  
40  
45  
50  
55  
60  
65  
70  
75  
80  
85  
90  
95  
100  
105  
110  
115  
120  
125  
130  
135  
140  
145  
150  
155  
160  
165  
170  
175  
180  
185  
190  
195  
200  
205  
210  
215  
220  
225  
230  
235  
240  
245  
250  
255  
260  
265  
270  
275  
280  
285  
290  
295  
300  
305  
310  
315  
320  
325  
330  
335  
340  
345  
350  
355  
360  
365  
370  
375  
380  
385  
390  
395  
400  
405  
410  
415  
420  
425  
430  
435  
440  
445  
450  
455  
460  
465  
470  
475  
480  
485  
490  
495  
500  
505  
510  
515  
520  
525  
530  
535  
540  
545  
550  
555  
560  
565  
570  
575  
580  
585  
590  
595  
600  
605  
610  
615  
620  
625  
630  
635  
640  
645  
650  
655  
660  
665  
670  
675  
680  
685  
690  
695  
700  
705  
710  
715  
720  
725  
730  
735  
740  
745  
750  
755  
760  
765  
770  
775  
780  
785  
790  
795  
800  
805  
810  
815  
820  
825  
830  
835  
840  
845  
850  
855  
860  
865  
870  
875  
880  
885  
890  
895  
900  
905  
910  
915  
920  
925  
930  
935  
940  
945  
950  
955  
960  
965  
970  
975  
980  
985  
990  
995  
1000  
1005  
1010  
1015  
1020  
1025  
1030  
1035  
1040  
1045  
1050  
1055  
1060  
1065  
1070  
1075  
1080  
1085  
1090  
1095  
1100  
1105  
1110  
1115  
1120  
1125  
1130  
1135  
1140  
1145  
1150  
1155  
1160  
1165  
1170  
1175  
1180  
1185  
1190  
1195  
1200  
1205  
1210  
1215  
1220  
1225  
1230  
1235  
1240  
1245  
1250  
1255  
1260  
1265  
1270  
1275  
1280  
1285  
1290  
1295  
1300  
1305  
1310  
1315  
1320  
1325  
1330  
1335  
1340  
1345  
1350  
1355  
1360  
1365  
1370  
1375  
1380  
1385  
1390  
1395  
1400  
1405  
1410  
1415  
1420  
1425  
1430  
1435  
1440  
1445  
1450  
1455  
1460  
1465  
1470  
1475  
1480  
1485  
1490  
1495  
1500  
1505  
1510  
1515  
1520  
1525  
1530  
1535  
1540  
1545  
1550  
1555  
1560  
1565  
1570  
1575  
1580  
1585  
1590  
1595  
1600  
1605  
1610  
1615  
1620  
1625  
1630  
1635  
1640  
1645  
1650  
1655  
1660  
1665  
1670  
1675  
1680  
1685  
1690  
1695  
1700  
1705  
1710  
1715  
1720  
1725  
1730  
1735  
1740  
1745  
1750  
1755  
1760  
1765  
1770  
1775  
1780  
1785  
1790  
1795  
1800  
1805  
1810  
1815  
1820  
1825  
1830  
1835  
1840  
1845  
1850  
1855  
1860  
1865  
1870  
1875  
1880  
1885  
1890  
1895  
1900  
1905  
1910  
1915  
1920  
1925  
1930  
1935  
1940  
1945  
1950  
1955  
1960  
1965  
1970  
1975  
1980  
1985  
1990  
1995  
2000  
2005  
2010  
2015  
2020  
2025  
2030  
2035  
2040  
2045  
2050  
2055  
2060  
2065  
2070  
2075  
2080  
2085  
2090  
2095  
2100  
2105  
2110  
2115  
2120  
2125  
2130  
2135  
2140  
2145  
2150  
2155  
2160  
2165  
2170  
2175  
2180  
2185  
2190  
2195  
2200  
2205  
2210  
2215  
2220  
2225  
2230  
2235  
2240  
2245  
2250  
2255  
2260  
2265  
2270  
2275  
2280  
2285  
2290  
2295  
2300  
2305  
2310  
2315  
2320  
2325  
2330  
2335  
2340  
2345  
2350  
2355  
2360  
2365  
2370  
2375  
2380  
2385  
2390  
2395  
2400  
2405  
2410  
2415  
2420  
2425  
2430  
2435  
2440  
2445  
2450  
2455  
2460  
2465  
2470  
2475  
2480  
2485  
2490  
2495  
2500  
2505  
2510  
2515  
2520  
2525  
2530  
2535  
2540  
2545  
2550  
2555  
2560  
2565  
2570  
2575  
2580  
2585  
2590  
2595  
2600  
2605  
2610  
2615  
2620  
2625  
2630  
2635  
2640  
2645  
2650  
2655  
2660  
2665  
2670  
2675  
2680  
2685  
2690  
2695  
2700  
2705  
2710  
2715  
2720  
2725  
2730  
2735  
2740  
2745  
2750  
2755  
2760  
2765  
2770  
2775  
2780  
2785  
2790  
2795  
2800  
2805  
2810  
2815  
2820  
2825  
2830  
2835  
2840  
2845  
2850  
2855  
2860  
2865  
2870  
2875  
2880  
2885  
2890  
2895  
2900  
2905  
2910  
2915  
2920  
2925  
2930  
2935  
2940  
2945  
2950  
2955  
2960  
2965  
2970  
2975  
2980  
2985  
2990  
2995  
3000  
3005  
3010  
3015  
3020  
3025  
3030  
3035  
3040  
3045  
3050  
3055  
3060  
3065  
3070  
3075  
3080  
3085  
3090  
3095  
3100  
3105  
3110  
3115  
3120  
3125  
3130  
3135  
3140  
3145  
3150  
3155  
3160  
3165  
3170  
3175  
3180  
3185  
3190  
3195  
3200  
3205  
3210  
3215  
3220  
3225  
3230  
3235  
3240  
3245  
3250  
3255  
3260  
3265  
3270  
3275  
3280  
3285  
3290  
3295  
3300  
3305  
3310  
3315  
3320  
3325  
3330  
3335  
3340  
3345  
3350  
3355  
3360  
3365  
3370  
3375  
3380  
3385  
3390  
3395  
3400  
3405  
3410  
3415  
3420  
3425  
3430  
3435  
3440  
3445  
3450  
3455  
3460  
3465  
3470  
3475  
3480  
3485  
3490  
3495  
3500  
3505  
3510  
3515  
3520  
3525  
3530  
3535  
3540  
3545  
3550  
3555  
3560  
3565  
3570  
3575  
3580  
3585  
3590  
3595  
3600  
3605  
3610  
3615  
3620  
3625  
3630  
3635  
3640  
3645  
3650  
3655  
3660  
3665  
3670  
3675  
3680  
3685  
3690  
3695  
3700  
3705  
3710  
3715  
3720  
3725  
3730  
3735  
3740  
3745  
3750  
3755  
3760  
3765  
3770  
3775  
3780  
3785  
3790  
3795  
3800  
3805  
3810  
3815  
3820  
3825  
3830  
3835  
3840  
3845  
3850  
3855  
3860  
3865  
3870  
3875  
3880  
3885  
3890  
3895  
3900  
3905  
3910  
3915  
3920  
3925  
3930  
3935  
3940  
3945  
3950  
3955  
3960  
3965  
3970  
3975  
3980  
3985  
3990  
3995  
4000  
4005  
4010  
4015  
4020  
4025  
4030  
4035  
4040  
4045  
4050  
4055  
4060  
4065  
4070  
4075  
4080  
4085  
4090  
4095  
4100  
4105  
4110  
4115  
4120  
4125  
4130  
4135  
4140  
4145  
4150  
4155  
4160  
4165  
4170  
4175  
4180  
4185  
4190  
4195  
4200  
4205  
4210  
4215  
4220  
4225  
4230  
4235  
4240  
4245  
4250  
4255  
4260  
4265  
4270  
4275  
4280  
4285  
4290  
4295  
4300  
4305  
4310  
4315  
4320  
4325  
4330  
4335  
4340  
4345  
4350  
4355  
4360  
4365  
4370  
4375  
4380  
4385  
4390  
4395  
4400  
4405  
4410  
4415  
4420  
4425  
4430  
4435  
4440  
4445  
4450  
4455  
4460  
4465  
4470  
4475  
4480  
4485  
4490  
4495  
4500  
4505  
4510  
4515  
4520  
4525  
4530  
4535  
4540  
4545  
4550  
4555  
4560  
4565  
4570  
4575  
4580  
4585  
4590  
4595  
4600  
4605  
4610  
4615  
4620  
4625  
4630  
4635  
4640  
4645  
4650  
4655  
4660  
4665  
4670  
4675  
4680  
4685  
4690  
4695  
4700  
4705  
4710  
4715  
4720  
4725  
4730  
4735  
4740  
4745  
4750  
4755  
4760  
4765  
4770  
4775  
4780  
4785  
4790  
4795  
4800  
4805  
4810  
4815  
4820  
4825  
4830  
4835  
4840  
4845  
4850  
4855  
4860  
4865  
4870  
4875  
4880  
4885  
4890  
4895  
4900  
4905  
4910  
4915  
4920  
4925  
4930  
4935  
4940  
4945  
4950  
4955  
4960  
4965  
4970  
4975  
4980  
4985  
4990  
4995  
5000  
5005  
5010  
5015  
5020  
5025  
5030  
5035  
5040  
5045  
5050  
5055  
5060  
5065  
5070  
5075  
5080  
5085  
5090  
5095  
5100  
5105  
5110  
5115  
5120  
5125  
5130  
5135  
5140  
5145  
5150  
5155  
5160  
5165  
5170  
5175  
5180  
5185  
5190  
5195  
5200  
5205  
5210  
5215  
5220  
5225  
5230  
5235  
5240  
5245  
5250  
5255  
5260  
5265  
5270  
5275  
5280  
5285  
5290  
5295  
5300  
5305  
5310  
5315  
5320  
5325  
5330  
5335  
5340  
5345  
5350  
5355  
5360  
5365  
5370  
5375  
5380  
5385  
5390  
5395  
5400  
5405  
5410  
5415  
5420  
5425  
5430  
5435  
5440  
5445  
5450  
5455  
5460  
5465  
5470  
5475  
5480  
5485  
5490  
5495  
5500  
5505  
5510  
5515  
5520  
5525  
5530  
5535  
5540  
5545  
5550  
5555  
5560  
5565  
5570  
5575  
5580  
5585  
5590  
5595  
5600  
5605  
5610  
5615  
5620  
5625  
5630  
5635  
5640  
5645  
5650  
5655  
5660  
5665  
5670  
5675  
5680  
5685  
5690  
5695  
5700  
5705  
5710  
5715  
5720  
5725  
5730  
5735  
5740  
5745  
5750  
5755  
5760  
5765  
5770  
5775  
5780  
5785  
5790  
5795  
5800  
5805  
5810  
5815  
5820  
5825  
5830  
5835  
5840  
5845  
5850  
5855  
5860  
5865  
5870  
5875  
5880  
5885  
5890  
5895  
5900  
5905  
5910  
5915  
5920  
5925  
5930  
5935  
5940  
5945  
5950  
5955  
5960  
5965  
5970  
5975  
5980  
5985  
5990  
5995  
6000  
6005  
6010  
6015  
6020  
6025  
6030  
6035  
6040  
6045  
6050  
6055  
6060  
6065  
6070  
6075  
6080  
6085  
6090  
6095  
6100  
6105  
6110  
6115  
6120  
6125  
6130  
6135  
6140  
6145  
6150  
6155  
6160  
6165  
6170  
6175  
6180  
6185  
6190  
6195  
6200  
6205  
6210  
6215  
6220  
6225  
6230  
6235  
6240  
6245  
6250  
6255  
6260  
6265  
6270  
6275  
6280  
6285  
6290  
6295  
6300  
6305  
6310  
6315  
6320  
6325  
6330  
6335  
6340  
6345  
6350  
6355  
6360  
6365  
6370  
6375  
6380  
6385  
6390  
6395  
6400  
6405  
6410  
6415  
6420  
6425  
6430  
6435  
6440  
6445  
6450  
6455  
6460  
6465  
6470  
6475  
6480  
6485  
6490  
6495  
6500  
6505  
6510  
6515  
6520  
6525  
6530  
6535  
6540  
6545  
6550  
6555  
6560  
6565  
6570  
6575  
6580  
6585  
6590  
6595  
6600  
6605  
6610  
6615  
6620  
6625  
6630  
6635  
6640  
6645  
6650  
6655  
6660  
6665  
6670  
6675  
6680  
6685  
6690  
6695  
6700  
6705  
6710  
6715  
6720  
6725  
6730  
6735  
6740  
6745  
6750  
6755  
6760  
6765  
6770  
6775  
6780  
6785  
6790  
6795  
6800  
6805  
6810  
6815  
6820  
6825  
6830  
6835  
6840  
6845  
6850  
6855  
6860  
6865  
6870  
6875  
6880  
6885  
6890  
6895  
6900  
6905  
6910  
6915  
6920  
6925  
6930  
6935  
6940  
6945  
6950  
6955  
6960  
6965  
6970  
6975  
6980  
6985  
6990  
6995  
7000  
7005  
7010  
7015  
7020  
7025  
7030  
7035  
7040  
7045  
7050  
7055  
7060  
7065  
7070  
7075  
7080  
7085  
7090  
7095  
7100  
7105  
7110  
7115  
7120  
7125  
7130  
7135  
7140  
7145  
7150  
7155  
7160  
7165  
7170  
7175  
7180  
7185  
7190  
7195  
7200  
7205  
7210  
7215  
7220  
7225  
7230  
7235  
7240  
7245  
7250  
7255  
7260  
7265  
7270  
7275  
7280  
7285  
7290  
7295  
7300  
7305  
7310  
7315  
7320  
7325  
7330  
7335  
7340  
7345  
7350  
7355  
7360  
7365  
7370  
7375  
7380  
7385  
7390  
7395  
7400  
7405  
7410  
7415  
7420  
7425  
7430  
7435  
7440  
7445  
7450  
7455  
7460  
7465  
7470  
7475  
7480  
7485  
7490  
7495  
7500  
7505  
7510  
7515  
7520  
7525  
7530  
7535  
7540  
7545  
7550  
7555  
7560  
7565  
7570  
7575  
7580  
7585  
7590  
7595  
7600  
7605  
7610  
7615  
7620  
7625  
7630  
7635  
7640  
7645  
7650  
7655  
7660  
7665  
7670  
7675  
7680  
7685  
7690  
7695  
7700  
7705  
7710  
7715  
7720  
7725  
7730  
7735  
7740  
7745  
7750  
7755  
7760  
7765  
7770  
7775  
7780  
7785  
7790  
7795  
7800  
7805  
7810  
7815  
7820  
7825  
7830  
7835  
7840  
7845  
7850  
7855  
7860  
7865  
7870  
7875  
7880  
7885  
7890  
7895  
7900  
7905  
7910  
7915  
7920  
7925  
7930  
7935  
7940  
7945  
7950  
7955  
7960  
7965  
7970  
7975  
7980  
7985  
7990  
7995  
8000  
8005  
8010  
8015  
8020  
8025  
8030  
8035  
8040  
8045  
8050  
8055  
8060  
8065  
8070  
8075  
8080  
8085  
8090  
8095  
8100  
8105  
8110  
8115  
8120  
8125  
8130  
8135  
8140  
8145  
8150  
8155  
8160  
8165  
8170  
8175  
8180  
8185  
8190  
8195  
8200  
8205  
8210  
8215  
8220  
8225  
8230  
8235  
8240  
8245  
8250  
8255  
8260  
8265  
8270  
8275  
8280  
8285  
8290  
8295  
8300  
8305  
8310  
8315  
8320  
8325  
8330  
8335  
8340  
8345  
8350  
8355  
8360  
8365  
8370  
8375  
8380  
8385  
8390  
8395  
8400  
8405  
8410  
8415  
8420  
8425  
8430  
8435  
8440  
8445  
8450  
8455  
8460  
8465  
8470  
8475  
8480  
8485  
8490  
8495  
8500  
8505  
8510  
8515  
8520  
8525  
8530  
8535  
8540  
8545  
8550  
8555  
8560  
8565  
8570  
8575  
8580  
8585  
8590  
8595  
8600  
8605  
8610  
8615  
8620  
8625  
8630  
8635  
8640  
8645  
8650  
8655  
8660  
8665  
8670  
8675  
8680  
8685  
8690  
8695  
8700  
8705  
8710  
8715  
8720  
8725  
8730  
8735  
8740  
8745  
8750  
8755  
8760  
8765  
8770  
8775  
8780  
8785  
8790  
8795  
8800  
8805  
8810  
8815  
8820  
8825  
8830  
8835  
8840  
8845  
8850  
8855  
8860  
8865  
8870  
8875  
8880  
8885  
8890  
8895  
8900  
8905  
8910  
8915  
8920  
8925  
8930  
8935  
8940  
8945  
8950  
8955  
8960  
8965  
8970  
8975  
8980  
8985  
8990  
8995  
9000  
9005  
9010  
9015  
9020  
9025  
9030  
9035  
9040  
9045  
9050  
9055  
9060  
9065  
9070  
9075  
9080  
9085  
9090  
9095  
9100  
9105  
9110  
9115  
9120  
9125  
9130  
9135  
9140  
9145  
9150  
9155  
9160  
9165  
9170  
9175  
9180  
9185  
9190  
9195  
9200  
9205  
9210  
9215  
9220  
9225  
9230  
9235  
9240  
9245  
9250  
9255  
9260  
9265  
9270  
9275  
9280  
9285  
9290  
9295  
9300  
9305  
9310  
9315  
9320  
9325  
9330  
9335  
9340  
9345  
9350  
9355  
9360  
9365  
9370  
9375  
9380

## [Surface Hardness]

The surface hardness was tested according to the pencil scratch test for paint film of JIS K5401-1969.

## [Cracking]

Occurrence of cracking at the surface of the recording medium was examined visually. The recording medium was evaluated to be "good" when no cracking was observed; to be "fair" when cracking was observed locally; and to be "poor" when cracking occurs over the entire surface.

## [Circularity]

Bk printing was conducted dot by dot by using the same ink jet printer and the same ink as the ones used in the above ink absorbency test. The major diameter D and the minor diameter d of one dot was measured by microscopy. The ratio of d/D was taken as the measure of the circularity.

## [Gloss]

The gloss of the recording medium at the non-printed area was measured by a gloss meter (Gloss Checker-IG-320, Horiba Seisakusho K.K.).

## [Water Fastness]

Single color solid-printing was conducted by using the same ink jet printer and the same ink as the ones used in the above ink absorbency test. The printed recording medium was immersed in flowing water for 3 minutes, and was air-dried. The water-resistance was represented by the equation below.

$$\text{Water resistance} = \frac{\text{Image density after water immersion}}{\text{Image density before water immersion}} \times 100$$

The recording medium was evaluated to be "good" when the water resistance was higher than 95, to be "fair" when the resistance was in the range of from 88 to 95, and to be "poor" when the resistance was lower than 88.

## [Light-fastness]

Bk single color solid-printing was conducted with the same ink-jet printer and the same ink in the above ink absorbency test. The ink was used in an amount of 100%. Thereafter, the printed recording medium was left standing at room temperature. The color tone (L\*) of the printed area was measured one day and 30 days after the printing, and the change ratio was derived. The recording medium was evaluated to be "good" when the change ratio was not more than  $\pm 10\%$ , to be "fair" when it was not more than  $\pm 20\%$ , and to be "poor" when it was more than  $\pm 20\%$ .

## [Migration]

One-dot printing of single color was conducted with the same ink-jet printer and the same ink as the ones used in the above ink absorbency test. The major diameters of the ink dots were measured one day and 30 days after the printing. The migration of the ink is prescribed by the equation below:

$$\text{Migration} = \frac{\text{Major diameter after 30 days}}{\text{Major diameter after one day}} \times 100$$

The recording medium was evaluated to be "good" in view of absence of migration of ink when the above value of migration was less than 105, to be "fair" when it was in the range of from 105 to 110, and to be "poor" when it was more than 110.

## EXAMPLES 1 to 4

Aluminum dodecyloxide was prepared according to the method described in U.S. Pat. No. 4,242,271. Then the resulting aluminum dodecyloxide was hydrolyzed into alumina in a slurry state according to the method described in

U.S. Pat. No. 4,202,870. To this alumina slurry, water was added to dilute it to the content of solid alumina hydrate of boehmite structure of 7.9% in the slurry. The alumina slurry showed a pH of 9.5. The pH was adjusted by adding 3.9% nitric acid solution. The slurry was aged under the conditions shown in Table 1 to obtain colloidal sols. This colloidal sols were spray-dried at 85° C. to obtain samples of powdery alumina hydrate of boehmite structure.

TABLE 1

|                                               | Aging Conditions of Alumina hydrate |      |      |      |
|-----------------------------------------------|-------------------------------------|------|------|------|
|                                               | Example No.                         |      |      |      |
|                                               | 1                                   | 2    | 3    | 4    |
| pH before aging                               | 6.6                                 | 6.6  | 6.8  | 6.4  |
| Aging temperature (° C.)                      | 48                                  | 49   | 50   | 35   |
| Aging period (days)                           | 14                                  | 16   | 18   | 16   |
| Aging apparatus                               | Oven                                | Oven | Oven | Oven |
| Crystallinity                                 | 20.2                                | 31.0 | 45.5 | 26.1 |
| BET specific surface area (m <sup>2</sup> /g) | 200                                 | 180  | 210  | 230  |
| Pore volume (cm <sup>3</sup> /g)              | 0.70                                | 0.75 | 0.71 | 0.68 |

The alumina hydrate of boehmite structure was dispersed in deionized water at a concentration of 17% by weight to obtain an alumina liquid dispersion. Separately, polyvinyl alcohol (trade name: Gosenol NH18 (hereinafter referred to as "PVA"), Nippon Gosei Kagaku K.K.) was mixed with deionized water at a concentration of 17% by weight to obtain a PVA solution. The alumina liquid dispersion and the PVA solution were mixed at a mixing ratio of 18:1 to obtain a coating liquid. This coating liquid was applied onto a resin-coated paper sheet by means of an extrusion coater at a coating temperature of 100° C. under shearing stress of 7.5 N/m<sup>2</sup> (75 dyn/cm<sup>2</sup>), and was delivered without blowing of drying air for one second to thicken and set the coating layer by utilizing thixotropy. Then the coating layer was dried for 30 seconds in an environment of relative humidity of 40% at a temperature shown in Table 2. The resulting recording medium was evaluated for the printing properties, etc. The evaluation results are shown in Table 2.

TABLE 2

|                                               | Evaluation results |      |      |      |
|-----------------------------------------------|--------------------|------|------|------|
|                                               | Example No.        |      |      |      |
|                                               | 1                  | 2    | 3    | 4    |
| Drying temperature (° C.)                     | 72                 | 80   | 90   | 72   |
| Crystallinity                                 | 19.8               | 32.2 | 47.5 | 28.1 |
| BET specific surface area (m <sup>2</sup> /g) | 180                | 165  | 185  | 195  |
| Pore volume (cm <sup>3</sup> /g)              | 0.50               | 0.58 | 0.56 | 0.51 |
| Ink Absorbency                                | Good               | Good | Good | Good |
| Ink absorption rate (seconds)                 | <10                | <10  | <10  | <10  |
| Surface hardness                              | HB                 | H    | H    | H    |
| Cracking                                      | Fair               | Good | Good | Good |

## EXAMPLE 5

A recording medium (before heating) was prepared in the same manner as in Examples 1 to 4 except that the aging conditions and drying conditions of the alumina hydrate were changed as shown in Table 3, the drying temperature was 68° C., the drying time was 30 seconds and the relative humidity was 50%. The resulting recording medium was

further heated for 30 minutes in an oven kept at a temperature of 80° C. and a relative humidity of 12% (recording medium after heating). The properties of the recording medium before and after heating are shown in Table 4. The heating treatment of the recording medium in this Example increases the crystallinity thereof, and thereby improving the ink absorbency, as shown in Table 4.

TABLE 3

| Aging conditions of Alumina hydrate in Examples 5, and 6-11 |      |      |      |
|-------------------------------------------------------------|------|------|------|
| Example No.                                                 |      |      |      |
|                                                             | 5    | 6-10 | 11   |
| pH before aging                                             | 6.4  | 6.3  | 6.1  |
| Aging temperature (° C.)                                    | 32   | 34   | 33   |
| Aging period (days)                                         | 15   | 18   | 16   |
| Aging apparatus                                             | Oven | Oven | Oven |
| Crystallinity                                               | 10.0 | 47.2 | 12.0 |
| BET specific surface area (m <sup>2</sup> /g)               | 220  | 235  | 230  |
| Pore volume (cm <sup>3</sup> /g)                            | 0.73 | 0.75 | 0.71 |

TABLE 4

| Evaluation Results in Example 5               |                |               |
|-----------------------------------------------|----------------|---------------|
|                                               | Before heating | After heating |
| Crystallinity                                 | 10.0           | 19.0          |
| Parallelization degree                        | 2.2            | 2.2           |
| BET specific surface area (m <sup>2</sup> /g) | 190            | 190           |
| Pore volume (cm <sup>3</sup> /g)              | 0.56           | 0.56          |
| Ink Absorbency                                | Fair           | Good          |
| Ink absorption rate (seconds)                 | 17             | <10           |
| Surface hardness                              | F              | H             |
| Cracking                                      | Fair           | Good          |
| Circularity                                   | 0.89           | 0.87          |
| Gloss                                         | 52             | 53            |

## EXAMPLES 6 to 10

Alumina hydrate liquid dispersions were prepared in the same manner as in Examples 1-4 except that the aging conditions and drying conditions were changed as shown in Table 3. The liquid dispersion was applied by means of an extrusion coater and dried. The shearing stress given to the coating liquid was adjusted to be 0.2 N/m<sup>2</sup> (Example 6), 6.0 N/m<sup>2</sup> (Example 7), 10.0 N/m<sup>2</sup> (Example 8), 14.0 N/m<sup>2</sup> (Example 9), and 18.0 N/m<sup>2</sup> (Example 10) respectively by changing the slit width and the extrusion pressure. The amount of the coating was 6 g/m<sup>2</sup> in each Example.

The coating was conducted at a rate of 1 m/s. The coated material was delivered without blowing of drying air for one second after the coating application to thicken and set the coating by utilizing thixotropy of the coating liquid, and then it was dried for 20 seconds at 90° C. at a relative humidity of 40%.

The resulting recording mediums were evaluated for printing properties. The results are shown in Table 5. The recording mediums prepared in these Examples changed their parallelization degree depending on the shearing stress given to the coating liquid, thereby changing the gloss.

TABLE 5

| 5                                             | Evaluation Results in Examples 6-10 |      |      |      |      |
|-----------------------------------------------|-------------------------------------|------|------|------|------|
|                                               | Example No.                         |      |      |      |      |
|                                               | 6                                   | 7    | 8    | 9    | 10   |
| Shearing stress (N/m <sup>2</sup> )           | 0.2                                 | 6.0  | 10.0 | 14.0 | 18.0 |
| Parallelization degree                        | 2.2                                 | 3.3  | 3.5  | 3.1  | 2.1  |
| BET specific surface area (m <sup>2</sup> /g) | 193                                 | 193  | 193  | 193  | 193  |
| Pore volume (cm <sup>3</sup> /g)              | 0.57                                | 0.57 | 0.57 | 0.57 | 0.57 |
| Circularity                                   | 0.88                                | 0.92 | 0.95 | 0.93 | 0.87 |
| Gloss                                         | 53                                  | 62   | 68   | 59   | 51   |

## EXAMPLE 11

25 Alumina hydrate liquid dispersion was prepared in the same manner as in Example 1 except that the aging conditions and the drying conditions were changed as shown in Table 3. With this liquid dispersion, a recording medium was prepared in the same manner as in Example 1 except that the relative humidity was changed to 15%. The evaluation results are shown in Table 6. The alumina hydrate in the recording medium prepared in this Example had higher crystallinity, and thereby the ink absorbency was improved as shown in Table 6.

TABLE 6

| 30 | Evaluation Results in Example 11              |      |
|----|-----------------------------------------------|------|
|    | Example 11                                    |      |
|    | Crystallinity                                 | 20.0 |
| 40 | BET specific surface area (m <sup>2</sup> /g) | 195  |
|    | Pore volume (cm <sup>3</sup> /g)              | 0.56 |
|    | Ink Absorbency                                | Good |
|    | Ink absorption rate                           | Good |
|    | Surface hardness                              | H    |
| 45 | Cracking                                      | Good |

## EXAMPLES 12 to 15

50 Alumina hydrate liquid dispersions were prepared in the same manner as in Examples 1-4 except that the aging conditions and drying conditions for the alumina hydrate of boehmite structure were changed as shown in Table 7. The liquid dispersions were applied and dried respectively by means of a kiss-roll coater. The shearing stresses given to the liquid dispersions are shown in Table 7. The shearing stress 55 was adjusted by changing the slit width and the extrusion pressure of the coating head. The amount of the coating was 7 g/m<sup>2</sup> in each Example. The coating was conducted at a rate of 0.8 m/s. The coated material was delivered without blowing drying air for one second after the coating application to thicken and set the coating by utilizing thixotropy of the coating liquid, then it was dried for 25 seconds at 85° C. and at a relative humidity of 35%.

Table 8 shows the results of the evaluation of the resulting recording medium.

TABLE 7

| Aging and Coating Conditions for Alumina hydrate |             |      |      |      |
|--------------------------------------------------|-------------|------|------|------|
|                                                  | Example No. |      |      |      |
|                                                  | 12          | 13   | 14   | 15   |
| pH before aging                                  | 6.3         | 6.6  | 6.3  | 6.5  |
| Aging temperature (° C.)                         | 35          | 38   | 40   | 33   |
| Aging period (days)                              | 16          | 12   | 15   | 17   |
| Aging apparatus                                  | Oven        | Oven | Oven | Oven |
| Crystallinity                                    | 16.0        | 45.2 | 52.5 | 30.0 |
| Shearing stress (N/m <sup>2</sup> )              | 0.2         | 10.8 | 19.8 | 0.3  |
| BET specific surface area (m <sup>2</sup> /g)    | 225         | 215  | 210  | 220  |
| Pore volume (cm <sup>3</sup> /g)                 | 0.70        | 0.71 | 0.71 | 0.70 |

TABLE 8

| Evaluation Results in Examples 12-15          |             |      |      |      |
|-----------------------------------------------|-------------|------|------|------|
|                                               | Example No. |      |      |      |
|                                               | 12          | 13   | 14   | 15   |
| Crystallinity                                 | 16.5        | 45.3 | 52.6 | 28.6 |
| Parallelization degree                        | 1.6         | 1.8  | 2.6  | 1.7  |
| BET specific surface Area (m <sup>2</sup> /g) | 190         | 187  | 185  | 188  |
| Pore volume (cm <sup>3</sup> /g)              | 0.51        | 0.52 | 0.52 | 0.51 |
| Light fastness                                | Good        | Good | Good | Fair |
| Water fastness                                | Fair        | Good | Good | Good |
| Ink migration                                 | Good        | Good | Good | Good |

The present invention has the advantages listed below:

- (1) A recording medium having higher ink absorbency, absorbing ink at a higher rate, and having a higher surface hardness is obtained by adjusting the crystallinity of alumina hydrate in the recording medium to be within in the specified range.
- (2) A recording medium enabling higher circularity of printed dots and having higher gloss is obtained by adjusting the parallelization degree of alumina hydrate in the recording medium to be within the specified range.
- (3) A printed matter having better light fastness and water resistance and being less likely to cause migration of ink is obtained by adjusting the crystallinity and the parallelization degree respectively to be within the specified ranges.

What is claimed is:

1. A recording medium having a porous ink-receiving layer containing alumina hydrate of boehmite structure formed on a base material, said ink-receiving layer formed of a dried coating of a liquid dispersion of said alumina hydrate onto said base material, an amount of said dried coating ranging from 2 to 60 g/m<sup>3</sup>, and said ink-receiving layer having a total pore volume ranging from 0.1 to 1.0 cm<sup>3</sup>/g, wherein microcrystals of said alumina hydrate are directed to be parallel to a plane direction of said ink-receiving layer at a parallelization degree of not less than 1.5, wherein the maximum length or the maximum diameter of said microcrystals ranges from 1 to 50 nm, and the parallelization degree is defined by an equation:

$$\text{Parallelization degree} = \frac{\text{Intensity ratio for medium}}{\text{Intensity ratio for powder}}$$

5 wherein

$$\text{Intensity ratio for medium} = \frac{\text{Peak intensity for plane (020) of medium}}{\text{Peak intensity for plane (120) of medium}},$$

10 and

$$\text{Intensity ratio for powder} = \frac{\text{Peak intensity for plane (020) of powder}}{\text{Peak intensity for plane (120) of powder}};$$

15 wherein said peak intensities are measured for each of the planes of medium and powder from X-ray diffraction measurements of the ink-receiving layer of the recording medium, and a powder obtained by pulverizing the ink-receiving layer, respectively.

20 2. The recording medium according to one of claim 1, wherein said parallelization degree is not less than 2.

25 3. A recording medium having a porous ink-receiving layer containing alumina hydrate of boehmite structure formed on a base material, said ink-receiving layer formed

25 of a dried coating of a liquid dispersion of said alumina hydrate onto said base material, an amount of said dried coating ranging from 2 to 60 g/m<sup>3</sup>, and said ink-receiving layer having a total pore volume ranging from 0.1 to 1.0 cm<sup>3</sup>/g, the crystallinity of said alumina hydrate in said porous ink-receiving surface layer ranging from 15 to 80, and microcrystals of the alumina hydrate being directed to be parallel to a plane direction of said ink-receiving layer at a parallelization degree of not less than 1.5, wherein the maximum length or the maximum diameter of said microcrystals ranges from 1 to 50 nm, and the parallelization degree is defined by an equation:

$$\text{Parallelization degree} = \frac{\text{Intensity ratio for medium}}{\text{Intensity ratio for powder}}$$

40 wherein

$$\text{Intensity ratio for medium} = \frac{\text{Peak intensity for plane (020) of medium}}{\text{Peak intensity for plane (120) of medium}},$$

and

$$\text{Intensity ratio for powder} = \frac{\text{Peak intensity for plane (020) of powder}}{\text{Peak intensity for plane (120) of powder}};$$

50 wherein said peak intensities are measured for each of the planes of medium and powder from X-ray diffraction measurements of the ink-receiving layer of the recording medium, and a powder obtained by pulverizing the ink-receiving layer, respectively.

55 4. The recording medium according to one of claim 3, wherein the crystallinity of said alumina hydrate in said porous ink-receiving surface layer ranges from 20 to 70.

5. The recording medium according to one of claim 3, 60 wherein said parallelization degree is not less than 2.

6. A recording medium for ink-jet recording having a porous ink-receiving layer containing alumina hydrate of boehmite structure formed on a base material, said ink-receiving layer formed of a dried coating of a liquid dispersion of said alumina hydrate onto said base material, an amount of said dried coating ranging from 2 to 60 g/m<sup>3</sup>, and said ink-receiving layer having a total pore volume ranging

**17**

from 0.1 to 1.0 cm<sup>3</sup>/g, wherein microcrystals of said alumina hydrate are directed to be parallel to a plane direction of said ink-receiving layer at a parallelization degree of not less than 1.5, wherein the maximum length or the maximum diameter of said microcrystals ranges from 1 to 50 nm.

7. A recording medium for ink-jet recording having a porous ink-receiving layer containing alumina hydrate of boehmite structure formed on a base material, said ink-receiving layer formed of a dried coating of a liquid dispersion of said alumina hydrate onto said base material, an amount of said dried coating ranging from 2 to 60 g/m<sup>3</sup>, and

**18**

said ink-receiving layer having a total pore volume ranging from 0.1 to 1.0 cm<sup>3</sup>/g, said alumina hydrate having crystallinity ranging from 15 to 80, and microcrystals of the alumina hydrate being directed to be parallel to a plane direction of said ink-receiving layer at a parallelization degree of not less than 1.5, wherein the maximum length or the maximum diameter of said microcrystals ranges from 1 to 50 nm.

\* \* \* \* \*

UNITED STATES PATENT AND TRADEMARK OFFICE  
**CERTIFICATE OF CORRECTION**

PATENT NO. : 6,342,289 B1  
DATED : January 29, 2002  
INVENTOR(S) : Eguchi et al.

Page 1 of 1

It is certified that error appears in the above-identified patent and that said Letters Patent is hereby corrected as shown below:

Column 1.

Line 16, "Ink jet" should read -- Ink-jet --;  
Line 18, "a" (second occurrence) should be deleted, and "Ink jet" should read -- Ink-jet --;  
Line 44, "cracking" should be deleted; and  
Line 64, "A still" should read -- Still --.

Column 3.

Line 18, "an" should read -- one --;  
Line 36, "Al<sub>2</sub>O<sub>3-n</sub>(OH)<sub>2</sub>.mH<sub>2</sub>O" should read -- Al<sub>2</sub>O<sub>3-n</sub>(OH)<sub>2n</sub>.mH<sub>2</sub>O --; and  
Line 39, "case" should read -- cases --.

Column 4.

Line 19, "-The" should read -- The -- and should begin a new paragraph.

Column 5.

Line 42, "almina" should read -- alumina --; and  
Line 58, "the idea" should read -- an idea --.

Column 9.

Line 20, "serves" should read -- serve --.

Column 13.

Table 3, Title, "conditions" should read -- Conditions --, and "hydrate" should read -- Hydrate --.

Column 16.

Line 20, "claim 1" should read -- claim 1 or 6 --; and  
Lines 56 and 59, "claim 3" should read -- claim 3 or 7 --.

Signed and Sealed this

Twenty-seventh Day of May, 2003



JAMES E. ROGAN  
*Director of the United States Patent and Trademark Office*